# EUROPEAN PATENT APPLICATION

(11) **EP 1 338 212 A2**
(43) Date of publication of application: **27.08.2003**
(21) Application number: 03002757.7
(22) Date of filing: 06.02.2003
(51) Int. Cl.: A44B 18/00

(54) **Loop fastener member superior in durability**

(30) Priority: 26.02.2002 JP 2002049671
(71) Applicant: KURARAY CO., LTD., Kurashiki-City Okayama Prefecture 710 (JP)
(72) Inventor: Takaaki, Tanaka, Kita-ku, Osaka-City, Osaka (JP); Yukitoshi, Higashinaka, c/o Magictape Co., Ltd., Fukui-Pref. (JP); Takashi, Katayama, Kurashiki-City, Okayama-Pref. (JP)
(74) Representative: Strehl Schübel-Hopf & Partner

(57) **Abstract**

Provided is a loop fastener member of good durability, in which the loop fastening elements sink down little to deform even in washing and wet heat pressure treatment at high temperatures. The loop fastener member comprises loop fastening elements formed to rise from a base fabric, and the loop fastening elements are formed of polyamide fibers of which from 60 to 100 mol% of the dicarboxylic acid units are aromatic dicarboxylic acid units and from 60 to 100 mol% of the diamine units are C₆₋₁₂ aliphatic diamine units.

## Description

### BACKGROUND OF THE INVENTION

### Field of the Invention

The present invention relates to a separable fastener that comprises a large number of loop fastening elements formed to rise from a woven or knitted base fabric, more precisely to a loop fastener member of good durability that comprises loop fastening elements formed of specific polyamide fibers.

### Description of the Related Art

Separable fasteners in which hook fastening elements and loop fastening elements are engaged with each other to form fastening have been utilized in various applications.

The use of such separable fasteners is expanding these days. In one embodiment of using them, for example, one separable fastener of looped fastening elements (this will be hereinunder referred to as a loop fastener member) is formed in linen such as bed sheets, quilt covers, pillowcases and sofa covers, while the other separable fastener of hooked fastening elements (this will be hereinafter referred to as a hook fastener member) is formed on the surface of the bodies to be covered with such linen, such as beds, quilts, pillows and sofas, and the hook fastening elements are engaged with the loop fastening elements to thereby fix the covers to the bodies. The service embodiment of the type is now increasing.

In the field of such applications, the covers are repeatedly washed and ironed. Therefore, the loop fastening elements of the loop fastener member fitted to the covers must be flexible and resistant to deformation stress. However, when the covers with conventional loop fastener members fitted thereto are repeatedly ironed, or that is, subjected to wet heat treatment under pressure at around 150°C, the loop fastening elements formed to rise from the base fabric of the covers are greatly deformed to an unrestorable degree, and it therefore leads to a problem in that the loop fastening elements fall down (sink down) to the base fabric, not restored to their original condition, and the engaging force is significantly lowered.

To solve the problem, for example, a loop fastener member is proposed in JP-A 7-308727, in which the loop fastening elements of the loop fastener member are formed of a mixture of monofilaments and multifilaments.

Heretofore, loop filaments are formed of fibers of nylon 6 or nylon 66 in many cases. However, these nylon fibers are not resistant to heat, and this will be a cause of the above-mentioned problem. Accordingly, in JP-A 11-253209, proposed is a loop fastener member of which the loop fastening elements are formed of polytrimethylene terephthalate fibers, a type of polyester fibers. However, the loop fastener member proposed is still problematic in that its restorability from thermal deformation is unsatisfactory and the engaging force is greatly lowered through repeated ironing.

### SUMMARY OF THE INVENTION

An object of the invention is to provide a loop fastener member that is superior in durability to wet-heat pressure treatment at high temperatures.

We, the present inventors have assiduously studied to solve the problems noted above, and, as a result, have found that, when specific polyamide fibers are used for forming loop fastening elements, then a loop fastener member resistant to ironing can be obtained.

Specifically, the present invention is a loop fastener member that comprises loop fastening elements risen from a base fabric, wherein the loop fastening elements are formed of polyamide fibers of which from 60 to 100 mol% of the dicarboxylic acid units are aromatic dicarboxylic acid units and from 60 to 100 mol% of the diamine units are C₆₋₁₂ aliphatic diamine units.

### DESCRIPTION OF THE PREFERRED EMBODIMENTS

The polyamide for use in the invention is so designed that from 60 to 100 mol% of the dicarboxylic acid units thereof are aromatic dicarboxylic acid units and from 60 to 100 mol% of the diamine units thereof are C₆₋₁₂ aliphatic diamine units. Preferably, the polyamide principally comprises the above-mentioned aromatic dicarboxylic acid units and the above-mentioned aliphatic diamine units, and at least 10 % of its terminal groups are blocked. More preferably, the polyamide that satisfies the condition further satisfies an additional condition that, when measured in concentrated sulfuric acid at 30°C, its intrinsic viscosity [η] is from 0.4 to 30 dl/g.

Especially in the invention, it is desirable that the polyamide contains at least 75 mol% of aromatic dicarboxylic acid units for the dicarboxylic acid units thereof from the viewpoint of the wet heat resistance and the engaging force, and also the mechanical properties of the loop fastener member. The aromatic dicarboxylic acid includes, for example, terephthalicacid, isophthalic acid, sodiumsulfoisophthalate, 2,6-naphthalenedicarboxylic acid, 2,7-naphthalenedicarboxylic acid, 1,4-naphthalenedicarboxylic acid, 1,4-phenylenedioxydiacetic acid, 1,3-phenylenedioxydiacetic acid, diphenic acid, 4,4'-oxydibenzoic, acid, diphenylmethane-4,4'-dicarboxylic acid, diphenylsulfone-4,4'-dicarboxylic acid, and 4,4'-biphenyldicarboxylic acid. Preferred are terephthalic acid and 2,6-naphthalenedicarboxylic acid; and more preferred is terephthalic acid. More preferably, at least 80 mol% of the aromatic dicarboxylic acid is terephthalic acid; and most preferably, the aromatic dicarboxylic acid is substantially terephthalic acid alone.

Other dicarboxylic acids than the aromatic dicarboxylic acid are, for example, aliphatic dicarboxylic acids such as malonic acid, dimethylmalonic acid, succinic acid, 3,3-diethylsuccinic acid, glutaric acid, 2,2-dimethylglutaric acid, adipic acid, 2-methyladipic acid, trimethyladipic acid, pimelic acid, azelaic acid, sebacic acid, suberic acid; and alicyclic dicarboxylic acids such as 1,3-cyctopentanedicarboxylic acid, 1,4-cyclohexanedicarboxylic acid. One or more dicarboxylic acid units selected from these may be introduced into the polyamide as copolymer units. In addition, a polycarboxylic acid having three or more functional groups such as trimellitic acid, trimesic acid or pyromellitic acid may also be in the polyamide within a melt-spinnable range.

In addition, from 60 to 100 mol% of the diamine units of the polyamide for use in the invention must be C₆₋₁₂ aliphatic diamine units. Preferably, the polyamide contains at least 75 mol%, more preferably at least 90 mol% of C₆₋₁₂ aliphatic diamine. The C₆₋₁₂ aliphatic diamine units include those derived from aliphatic diamines such as 1,6-hexanediamine, 1,8-octanediamine, 1,9-nonanediamine, 1,10-decanediamine, 1,12-dodecanediamine, 2-methyl-1,5-pentanediamine, 3-methyl-1,5-pentanediamine, 2,2,4-trimethyl-1,6-hexanediamine, 2,4,4-trimethyl-1,6-hexanediamine, 2-methyl-1,8-octanediamine and 5-methyl-1,9-nonanediamine. Above all, preferred are 1,9-nonanediamine units in view of the deformation resistance and the durability of the loop fastener member; and more preferred is a combination of 1,9-nonanediamine units and 2-methyl-1,8-octanediamine units.

In the combination, the molar ratio of 1,9-nonanediamine units to 2-methyl-1,8-octanediamine units preferably falls between 9/1 and 1/9. More preferably, the combination of 1,9-nonanediamine units and 2-methyl-1,8-octanediamine units accounts for at 80 mol% of the C₆₋₁₂ aliphatic diamine units.

Examples of other diamines than the C₆₋₁₂ aliphatic diamines are aliphatic diamines, such as ethylenediamine, propylenediamine, tetramethylenediamine, pentamethylenediamine; alicyclic diamines such as cyclohexanediamine, methylcyclohexanediamine, isophoronediamine, and aromatic , diamines such as p-phenylenediamine, m-phenylenediamine, xylylenediamine, xylenediamine, 4,4'-diaminodiphenylmethane, 4,4'-diaminodiphenyl sulfone, 4,4'-diaminodiphenyl ether.

Especially in the invention, it is desirable that at least 10 %, more preferably at least 40 %, most preferably at least 70% of the terminal groups of the molecular chain of the polyamide are blocked with a terminal blocking agent. If the degree of terminal blocking of the polyamide for use in the invention is less than 10 %, the fibers formed may be discolored and their strength may be unsatisfactory. The degree of terminal blocking of the polyamide can be determined by counting the number of the terminal carboxyl groups, the number of the terminal amino groups and the number of the terminal groups blocked with a terminal blocking agents. It is desirable that, in view of its accuracy and simplicity, the number of the terminal groups is obtained by ¹H-NMR spectroscopy, by separately integrating the characteristic signals corresponding to the terminal groups.

Not specifically defined, the terminal blocking agent may be any and every compound reactive to the amino group or the carboxyl group of the polyamide terminal.

In view of their reactivity and the stability of the terminals blocked with them, preferred are monocarboxylic acids such as typically benzoic acid and monoamines; and more preferred are monocarboxylic acids as they are easy to handle. Apart from the above-mentioned compounds , also usable are acid anhydrides such as phthalic anhydride; monoisocyanates, mono-acid halides, monoesters, and monoalcohols.

Not also specifically defined, the polyamide for use in the invention may be produced in any known method. For example, it may be produced through solution polymerization or interfacial polymerization of starting materials of acid chlorides and diamines, or through melt polymerization, solid-phase polymerization or melt-extrusion polymerization of starting materials of dicarboxylic acids and diamines.

Preferably, the polyamide has, as the index of its molecular weight, an intrinsic viscosity [η] of from 0.6 to 2.0 dl/g, more preferably from 0.6 to 1.8 dl/g, most preferably from 0.7 to 1.5 dl/g measured in concentrated sulfuric acid at 30°C. Having the intrinsic viscosity falling within the range, the melt spinnability of the polyamide is good, and, in addition, the mechanical properties of the fibers to be made of it are good and the durability of the loop fastener member formed of the fibers is further improved.

If desired, the polyamide fibers to constitute the loop fastener member may contain colorants such as dye, pigment; and various stabilizers such as typically antioxidant and light stabilizer. In addition, their surfaces may be coated with a chemical having the ability to improve the lubricity of the fibers.

The loop fastener member of the invention is formed of the polyamide fibers mentioned above, and the fiber diameter may be from 20 to 100 µm. More preferably, however, for increasing the deformation resistance of the loop fastening elements not worsening the feel of the loop fastener member, from 10 to 90 single fibers each having a fiber diameter of from 40 to 90 µm are bundled up into multifilaments for forming the loop fastening elements The loop fastening elements-forming fibers are woven along with the other weft and warp to constitute the base fabric of the loop fastener member, and then back-coated and heat-set in an ordinary manner, and the process gives the loop fastener member of the invention. Needless-to-say, the other weft and warp may be formed of the the above-mentioned specific polyamide, or may be formed of any others polyamide fibers, polyester esters, other synthetic fibers, natural fibers, regenerated fibers, etc. Regarding their height, it is desirable that the loop fastening elements rise from the face of the base fabric by from 1 to 5 mm or so for preventing them from being deformed in wet heat pressure treatment.

The invention relates to a loop fastener member, and the loop fastener member of the invention is not meant to indicate a loop fastener member loop fastening elements alone but includes a hook-and-loop coexisting fastener that comprises both loop fastening elements and hook fastening elements formed on one and the same base fabric. This means that the loop fastener member of the invention encompasses any and every type of fastener member having loop fastening elements formed on a base fabric.

The loop fastener member of the invention has good durability and is especially favorable for clothing. In addition, the loop fastener member of the invention has high engaging force, and not only for clothing, it is also usable for bed sheets, quilt covers, pillowcases, sofa covers, etc.

### EXAMPLES

The invention is described in more detail with reference to the following Examples, which, however, are not intended to restrict the scope of the invention. The physical properties of the samples in the invention were measured according to the methods mentioned below.

### Intrinsic Viscosity [η] of Polyamide:

A sample having a predetermined concentration in concentrated sulfuric acid at 30°C is measured to obtain its inherent viscosity (ηinh). Its data are extrapolated to a concentration 0, and the resulting value is the intrinsic viscosity [η] of the sample.${\text{ηinh = [ln(t}}_{\text{1}} {\text{/t}}_{\text{0}} \text{)]/c}$ wherein ηinh indicates the inherent viscosity (dl/g) of the sample; t₀ indicates the flow down time (sec) of the solvent; t₁ indicates the flow down time (sec) of the sample solution; and c indicates the sample concentration (g/dl) in the solution.

### Durability to Wet Heat Pressure Treatment:

A loop fastener member (width 25 mm, length 100 mm) is sewed on a cotton fabric (mass per unit area 200 g/m²) to prepare a sample.

The sample is put into a domestic washing machine, and room-temperature tap water is put thereinto to have a bath ratio of 1:50. Further, a weak-alkaline synthetic detergent (Lion's Top (trade name)) is added to it in a ratio of 1 g/liter. This is continuously washed for 1 hour, then rinsed for 5 minutes and dewatered through centrtfugation for 5 minutes. Next, the sample is pressed with a Hoffman hot presser at 150°C for 5 minutes. This washing and pressing operation is one cycle. The sample is subjected to a predetermined number of the cycles. The engaging force of the loop fastener member of the sample is measured, tried with a hook fastener member (this comprises hook fastening elements of polyester monofilaments, having a fiber diameter of 0.20 mm, a height of the fastening elements of 1.80 mm, and a density of the fastening elements of 40/cm²). The engaging force is measured according to the method of JIS-L-3416, in which the peeling strength and the tensile shearing strength of the sample are measured.

A dicarboxylic acid component of terephthalic acid was polymerized with a diamine component of 1,9-nonanediamine and 2-methyl-1,8-octanediamine (molar ratio, 1:1) along with a terminal blocking agent of benzoic acid to obtain a polyamide having a degree of terminal blocking of 90 % and an intrinsic viscosity [η] of 0.8 dl/g.

The resulting polyamide was melt-spun into polyamide multifilaments having a fineness of 230 dtex/10 filaments (diameter of each fiber: 48 µm). These were looped on a base fabric of polyester multifilaments of 167 dtex/48 filaments for both the warp and the weft to fabricate a loop fastener member having a loop height of 2.89 mm and a loop density of 60 loops/cm².

The durability of the thus-obtained loop fastener member was evaluated according to the method mentioned above. The engaging force of the sample before washed and the engaging force thereof after 5 cycles were measured according to the above-mentioned method, and the force retention was obtained. The results are given in Table 1.

### Comparative Example 1:

A loop fastener member was fabricated, for which the loop yarn was polyester multifilaments having a fineness of 267 dtex/10 filaments and the warp and the weft of the base fabric were polyester multifilaments of 167 dtex/48 filaments. The loop height was 2.59 mm, and the loop density was 60 loops/cm². This was repeatedly washed and hot-pressed in the same manner as in Example 1, and its engaging force was measured. In addition, the engaging force retention was also evaluated. The results are given in Table 1.

### Comparative Example 2:

A loop fastener member was fabricated, for which the loop yarn was nylon-6 multifilaments having a fineness of 230 dtex/10 filaments and the warp and the weft of the base fabric were nylon-6 multifilaments of 156 dtex/12 filaments. The loop height was 2.47 mm, and the loop density was 60 loops/cm². This was repeatedly washed and hot-pressed in the same manner as in Example 1, and its engaging force was measured. In addition, the engaging force retention was also evaluated. The results are given in Table 1.

### Comparative Example 3:

A loop fastener member was fabricated, for which the loop yarn was nylon-66 multifilaments having a fineness of 300 dtex/16 filaments and the warp and the weft of the base fabric were nylon-66 multifilaments of 149 dtex/34 filaments. The loop height was 2.65 mm, and the loop density was 60 loops/cm². This was repeatedly washed and hot-pressed in the same manner as in Example 1, and its engaging force was measured. In addition, the engaging force retention was also evaluated. The results are given in Table 1.

**Table 1**

| | Tensile Shearing Strength (kg/cm²) | | Peeling Strength (g/cm) | |
|---|---|---|---|---|
| | before washed | after 5 cycles (force retention, %) | before washed | after 5 cycles (force retention, %) |
| Example 1 | 1.23 | 0.84 (68.3) | 154 | 120 (77.9) |
| Comparative Example 1 | 1.37 | 0.30 (21.9) | 169 | 68 (40.2) |
| Comparative Example 2 | 1.16 | 0.50 (43.1) | 129 | 86 (66.7) |
| Comparative Example 3 | 1.20 | 0.61 (50.8) | 157 | 100 (63.7) |

### Example 2:

A hook-and-loop coexisting fastener was fabricated, for which the warp and the weft of the base fabric were nylon-6 multifilaments having a fineness of 150 dtex/12 filaments, the loop yarn was the polyamide multifilaments used in Example 1, and the hook yarn was nylon-66 monofilaments having a fineness of 430 dtex. Thus obtained, the hook-and-loop coexisting fastener had a hook height of 2.05 mm, a hook density of 30 hooks/cm², a loop height of 2.45 mm, and a loop density of 40 loops/cm². This was washed in the same manner as in Example 1, and its engaging force was measured. The results are given in Table2.

### Comparative Example 4:

A hook-and-loop coexisting fastener was fabricated in the same manner as in Example 2, for which, however, the loop yarn was nylon-6 multifilaments having a fineness of 230 dtex/10 filaments. This was washed in the same manner as in Example 2, and its engaging force was measured. The results are given in Table 2.

**Table 2**

| | Tensile Shearing Strength (kg/cm²) | | Peeling Strength (g/cm) | |
|---|---|---|---|---|
| | before washed | after 5 cycles (force retention, %) %) | before washed | after 5 cycles (force retention, %) |
| Example 2 | 1.25 | 0.92 (73.6) | 140 | 120 (85.7) |
| Comparative Example 4 | 1.20 | 0.79 (65.8) | 130 | 98 (75.4) |

As described in detail hereinabove with reference to its preferred embodiments, the invention provides a loop fastener member of good durability, in which the loop yarn sinks down little even in washing and wet heat pressure treatment at high temperatures.

## Claims

1. A loop fastener member that comprises loop fastening elements risen from a base fabric, wherein the loop fastening elements are formed of polyamide fibers of which from 60 to 100 mol% of the dicarboxylic acid units are aromatic dicarboxylic acid units and from 60 to 100 mol% of the diamine units are C₆₋₁₂ aliphatic diamine units.
